

# UNITED STATES PATENT OFFICE.

GUY M. LAIRD, OF CHICAGO, ILLINOIS, ASSIGNOR OF ONE-HALF TO LEO B. LINCOLN, OF CHICAGO, ILLINOIS.

## ELECTRIC-RESISTANCE ELEMENT.

1,257,272.

Specification of Letters Patent.

Patented Feb. 19, 1918.

No Drawing.

Application filed May 19, 1916. Serial No. 98,674.

*To all whom it may concern:*

Be it known that I, GUY M. LAIRD, a citizen of the United States, residing at Chicago, county of Cook, State of Illinois, have 5 invented a certain new and useful Improvement in Electric-Resistance Elements, and declare the following to be a full, clear, and exact description of the same, such as will enable others skilled in the art to which it 10 pertains to make and use the same.

My invention or discovery consists in the production of a new electric resistance element composed of a metal which shall have the property of being particularly low in 15 electric conductivity, have a melting point exceeding that of pure copper, and be capable of resisting oxidation at all temperatures and under all conditions to which it needs to be subjected, while at the same time 20 possessing characteristics permitting it to be drawn or otherwise worked to form strips, strands or filaments; whereby highly efficient and extremely durable resistance elements result.

My invention or discovery consists simply in making an electric resistance element of an alloy of one or more of the members of the nickel group of metals (nickel, cobalt, and iron) with silicon. The addition of silicon to nickel, for example, raises the melting point of the latter and also the temperature at which oxidation will take place and at the same time lowers its electric conductivity, giving a resistance element very similar in essential characteristics to the nickel-

chromium resistance material now so largely used. To make the material more ductile than it would otherwise be, cobalt may be added. While the nickel or nickel and cobalt alloys will ordinarily be preferable, iron, 40 when alloyed with silicon will give excellent results, it being necessary of course that the iron be pure so that it will not oxidize under ordinary atmospheric conditions; pure iron being practically non-oxidizable at ordinary 45 temperatures and the addition of the silicon raising the melting point so that oxidation at high temperatures does not become appreciable until a much higher temperature is reached than will be the case with the iron 50 alone.

The amount of silicon employed will vary according to the service to which the resistance material is to be put. In some cases the silicon content will amount to only a few 55 per cent., while in others it may be as high as twenty-four per cent. Where the alloy is of nickel, cobalt and silicon, it may be stated as a general rule that the nickel content should be at least seventy-five per cent. 60 of the whole.

I claim:

An electric resistance element formed of an alloy of nickel, cobalt and silicon and containing at least seventy-five per cent. of 65 nickel.

In testimony whereof, I sign this specification.

GUY M. LAIRD.